

March 18, 1941.

E. C. GAERTNER

2,235,291

## METHOD OF PRODUCING HOLLOW CLAY TILE

Filed April 3, 1939

FIG. 1



FIG. 2



INVENTOR.  
EDWARD C. GAERTNER.  
ATTORNEY.  
Lockwood, Tolman & Galt.

## UNITED STATES PATENT OFFICE

2,235,291

## METHOD OF PRODUCING HOLLOW CLAY TILE

Edward C. Gaertner, Terre Haute, Ind., assignor, by mesne assignments, to Reconstruction Finance Corporation, Chicago, Ill., a corporation of the United States

Application April 3, 1939, Serial No. 265,690

3 Claims. (Cl. 25—156)

This invention relates to a method of producing a vitrified clay product.

The chief object of this invention is to eliminate in clay products for permanent, sanitary and decorative wall finish purposes, certain objections heretofore inherent therein and to obtain new and desirable features.

One of the chief objections to present clay ware is that it must be sold with certain tolerances, now accepted by the architects as a necessary evil. The present invention eliminates this objection.

Another chief objection to large size present clay ware is that it has plane distortion. The present invention eliminates this objection as well.

In addition to the aforesaid objections, present ware production has an unavoidable wastage incident to handling deformation that results in deformed finished ware unacceptable for normal use. The present invention reduces this objection to a minimum and to a calculatable positive amount, and at little additional cost as will hereinafter more fully appear.

The present invention is also capable of including a finished or glazed face, or faces, if, as and when desired.

The full nature of the invention will be understood from the accompanying drawing and the following description and claims:

In the drawing,

Fig. 1 is a perspective view of the vitrified "log" from which the finished clay units are fabricated.

Fig. 2 is a similar view of a modified form of log.

For a better understanding of this invention, it is set forth that heretofore clay ware has been produced in the approximate form and size in the "green" state and then burned to vitrification. Exposed surfaces may be supplied with glaze finish material and fused thereto in the initial burning of the unit.

The resulting ware, due to inherent shrinkage, will vary not only as to size but shape as well. Also the vitrified ware will have included therein all other deformations incident to "green" ware handling. This wastage alone is considerable and variable.

The present invention, in brief, contemplates the formation of a very large unit in "green" form, burning to vitrification, and then cutting to size and form. The log, when vitrified, is in such shape and size that it can be sawed with a minimum amount of wastage incident to truing and kerfing.

The ware may be of acoustical or glazed face character, as desired.

In the drawing, each figure is to scale. Fig. 1 illustrates in perspective a "log" which has been formed in the following manner:

The raw clay is processed in the usual manner and homogeneously mixed therewith is a combustible material in finely divided form. This may be coal, sawdust, corn husks, and the like.

This mixture is extruded from a die in the usual manner and the clay column is cut to the desired length.

By way of illustration, the length selected is such that when burned to vitrification, a 38" log provides a 36" length with finished end faces and which can be reduced to lengths of 3", 4", 6", 8", 12", 15" and 18", et cetera, lengths, providing the desired number of desired length units of ware. Of course, when cut to 3", 4", 6", 9", 12" and 18", the log will form a plurality of 15 like length units.

Similarly, the log when vitrified is about 16 $\frac{1}{4}$ " on a side. This provides units of 1 $\frac{1}{8}$ " and 3 $\frac{3}{4}$ " thickness and 12" in width and four corner units 1 $\frac{1}{8}$ " x 1 $\frac{1}{8}$ " finished two faces. The four 12" x 1 $\frac{1}{8}$ " side units are finished three faces. The three central 12" x 3 $\frac{3}{4}$ " units are finished four faces. The length of these several units may be that selected and as designated above.

The "green" log is burned to vitrification. In so doing, the combustible material is burned out leaving small voids in the ware providing a cellular ware suitable for acoustical purposes. Also this type of vitrified log readily lends itself to rapid reduction by a patentable sawing machine.

Inherently this machine includes a plurality of parallel sawing elements so that a plurality of cuttings can be simultaneously effected as the log or ware is presented thereto or the saws are caused to move into the work. Each saw cuts a kerf of not more than  $\frac{1}{16}$ " width and opposed faces are parallel, smooth and coplanar throughout.

It will be understood the rough log (vitrified) 40 in its exposed faces, ends, and edges contains all imperfections incident to the handling, et cetera, of the "green" log prior to and during vitrification. Also all deformation, such as due to shrinkage, plane distortion and the like during vitrification is, of course, multiplied in the resultant log by reason of its large size. For this reason large size standard ware is economically impossible to produce for structural use. This means more or larger mortar joints in the finished structure, 50 because of the use of smaller units in the present standard practice or the irregularities therein and especially units of larger sizes necessitate larger joints. The various designs of large cells in their arrangement permit the formation of 55 cavities resulting in light weight or non-solid cellular ware. This also facilitates and expedites the reduction of the log into finished units.

In Fig. 1, the unfinished vitrified log is designated by the letter A. The log is then simultane- 60

ously slabbed as indicated at B' and B<sup>2</sup>. These kerfs extend the full length of the log and full width of the same. This provides planks C' and C<sup>2</sup> and the intermediate portion C<sup>3</sup>.

5 Portion C<sup>3</sup> is then simultaneously kerfed as at D', D<sup>2</sup>, D<sup>3</sup> and D<sup>4</sup>. This forms two end planks E' and E<sup>2</sup> and three central units E<sup>3</sup>, E<sup>4</sup> and E<sup>5</sup>. The plank C' is kerfed at F' and F<sup>2</sup> forming unit G' and corner units G<sup>2</sup> and G<sup>3</sup>. Similarly, plank 10 C<sup>2</sup> is kerfed at H' and H<sup>2</sup> forming unit J' and corner units J<sup>2</sup> and J<sup>3</sup>.

All corner units are approximately 1 1/8" x 1 1/8". All plank units are approximately 1 1/8" x 12". The central units are exactly 3 3/4" x 12". Each 15 corner unit has no cavity. Each "plank" unit includes three sequentially arranged longitudinally aligned cavities K. Each of the master or central units includes three sequentially arranged and longitudinally aligned cavities L. Cavities K have one dimension, the same as cavities L. The other dimension obviously is less than half the other dimension of cavity L due to the necessity for providing an exterior wall.

All walls between finished faces and cavities 20 have sufficient thickness. These are not uniform in thickness because in the reduction of an "irregular" log to the true units, the cavities do not always exactly center in the unit.

Preferably, all these operations are performed 25 before the ends are trimmed and the trimmed lengths are reduced to proper length. The end cuttings are indicated by letters N' and N<sup>2</sup>, and the length cuttings by O' and O<sup>2</sup>. Herein such cuttings provide 12" length units.

30 Should the log have a deformity of an excessive size, it will be obvious that the particular plank unit or corner unit may be discarded. If the end be unduly deformed, it will be obvious the 36" length can be shifted from that end 40 toward the opposite end.

Also any standard 12" unit could be reduced to 3", 4", 6", 8" or 9" length for extra smaller size units, the deformed portion being discarded.

Each of the triple cavity units may be reduced 45 on the job by a smaller size saw to form single cavity and single and double cavity units. Also each central unit can be readily divided forming units finished on three faces and an unfinished and irregular fourth or back face. Such reductions are indicated by dotted lines P and Q in Fig. 1.

In Fig. 2 there is illustrated a modified form of log. Herein dual letters, similar to the single letters, are employed to designate parts, et cetera, 55 like or similar to those singularly designated in Fig. 1. For clearance, however, many reference letters are omitted in Fig. 2.

In Fig. 2 plank units EE' and EE<sup>2</sup> have end cavities KK' smaller than cavities KK. This 60 leaves an end portion RR at either end (the latter being illustrated) which may be reduced as at SS to provide an angular face, or faces, respectively.

In like manner, central units EE<sup>3</sup> and EE<sup>5</sup> have 65 cavities LL' smaller than cavities LL and one wall is biased as indicated at LL<sup>2</sup> providing portion TT at either or both ends (the latter being illustrated) which may be reduced as at UU to provide an angular face, or faces, respectively.

This brief reference to the form of log illustrated in Fig. 2 it is believed is sufficient for an 70 understanding of the invention, it being understood that log AA is fabricated in exactly the same manner as log A.

Whenever it is desired to provide glazed ware, 75 the units after formation to the size selected

have the faces to be coated supplied with glaze material which matures at a temperature below that of vitrification. Usually a filler coat and then a final coat is applied, the latter immediately following filler coat application. The coated ware is then fired at a temperature sufficient to mature the glaze finish but below that of vitrification, so that deformation of the unit is impossible. The breakage loss in handling is substantially the only loss which occurs and this negligible since 10 the ware is not "green." With but slight care, no wastage incidental to glazing will occur.

From the foregoing it will be obvious that from 15 the log approximately the maximum amount of surface ware, true to form and the like, can be obtained with a minimum of loss.

The ware factory can produce large numbers of logs and subsequently fabricate same to the desired and required sizes of units. This eliminates the necessity of carrying stocks of different vitreous clay ware, thereby reducing inventories and smoothing out the plant production curve. Other advantages and economies will be obvious from the foregoing.

A comparative table is set forth which is by no 20 means complete but the same is illustrative of the advantages of the present invention over the present standard practice.

| Characteristic                            | Present structural glazed ware (standard)                            | Invention ware                                                                           | 30 |
|-------------------------------------------|----------------------------------------------------------------------|------------------------------------------------------------------------------------------|----|
| Weight.....                               | Min. 27# per sq. ft. 4"                                              | Max. 13# per sq. ft. 4".                                                                 |    |
| Strength.....                             | Beyond all load bearing code requirements.                           | Beyond all load bearing code requirements.                                               | 35 |
| Size.....                                 | 2 1/4 x 8, 5 x 8, 5 x 12 and 8 x 16.                                 | All the foregoing plus 6 x 12, 12 x 12, 12 x 24, 12 x 36 and larger.                     |    |
| Size variation.....                       | Approx. 1/4" per lineal foot.                                        | Less than 1/32" in 36".                                                                  |    |
| Colors.....                               | Limited to those manufacturing at high temperatures.                 | Unlimited.                                                                               | 40 |
| Textures.....                             | All glazed textures.....                                             | All glazed textures plus an unglazed acoustical texture if desired.                      |    |
| Kiln recovery "A" grade of finished ware. | Max. 75%.....                                                        | Anticipated min. of 90%.                                                                 | 45 |
| Reclamation of off grade ware.            | Practically none. Sold at greatly reduced prices or as "grog."       | 75% by cutting defective portions out of full size and making intermediate usable sizes. |    |
| Delivery time from date of order.         | Generally 3 to 4 weeks unless tremendous inventories are carried.    | 7 days.                                                                                  | 50 |
| Inventories.....                          | Varies in "A" grade. Usually great volume of slow moving off grades. | Predetermined quantity of logs. Finished stock A grade on order only and no off grades.  |    |
| Packing.....                              | .....                                                                | 33% saving.                                                                              | 55 |
| Freight and carriage.                     | .....                                                                | Savings in direct relation to weight.                                                    |    |
| Damage in transit or on job.              | Practically total loss because of difficulty in cutting.             | High percentages reclaimed by easy cutting to short lengths.                             |    |
| Cutting or fabricating.                   | Slow and costly.....                                                 | Fast and at low cost.                                                                    | 60 |
| Mortar.....                               | 1/4" to 3/8"                                                         | 75% saving.                                                                              | 65 |
| Joint size.....                           | Relatively slow, account low absorption of bed.                      | Uniform 1/8" or less.                                                                    |    |
| Setting.....                              | In relation to size, the larger the unit the less per sq. ft.        | Fast because of high absorption of bed.                                                  |    |
| Cost of labor of setting.                 | In relation to size; the larger the unit the less per sq. ft.        | In relation to size; the larger the unit the less per sq. ft.                            | 65 |

A unit thus specifically described produces about 30 sq. ft. of wall surface, which with labor at 60-cents per hour, costs between \$3.25 and \$3.50 when properly cut and glazed, if desired. The usual cost for this amount of ware of transportation, selling and erection is about \$200. The usual cost of an equivalent amount of standard ware is between \$15.00 to \$18.00 although in a recent instance same was sold at \$12.00. If the 75

erection, et cetera, cost be assumed the same, although standard ware costs for loading, unloading and erection will be more than that of the present invention, and the lower price be used 5 for comparison, in situ, 30 sq. ft. of the invention will cost \$5.50 as against \$15.00. This saving means that this new ware is capable of competing on a more favorable basis with other structural constructions, such as brick, or tile covered 10 surfaces, or glass covered surfaces and in its own field will offer an enormous saving for those using this type of construction.

By the term "closed tubular" in the claims, it is to be understood that the tube forming opening 15 wall includes no lateral rupture or opening to the tubularity and does not refer to the ends of the tubular structure.

While the invention has been illustrated and described in great detail in the drawing and 20 foregoing description, the same is to be considered as illustrative and not restrictive in character.

The several modifications described herein as well as others which will readily suggest themselves to persons skilled in this art, all are considered to be within the broad scope of the invention, reference being had to the appended 25 claims.

The invention claimed is:

1. An improved method of producing struc-

tural clay ware and the like, including forming an elongated "green" log of a homogeneous mixture and the desired dimensions and including spaced cavities extending longitudinally therethrough, burning the log to vitrification to produce a readily severable product, and then longitudinally severing the log cavity forming wall between adjacent cavities without exposing the latter, and between the ends by sawing to form finished face, closed, tubular units, some of which 10 are all finished and others of which are finished on all but one or two faces.

2. A method as defined by claim 1, characterized by arranging the cavities in the log such that upon severance into units each unit except the 15 corner unit includes a plurality of sequentially aligned cavities, and then longitudinally severing each unit between adjacent cavities without exposing the latter to form smaller, finished face, 20 closed, tubular units.

3. A method as defined by claim 1, characterized by arranging the cavities in the log such that upon severance into units each unit except the corner units includes a plurality of sequentially aligned cavities, certain unit end cavities 25 being smaller than others, and then bias severing the unit adjacent the smaller cavity without exposing same.

EDWARD C. GAERTNER.